

Sept. 21, 1926.

1,600,782

W. P. WITHEROW

DIE ROLL AND DIE ROLLING

Filed Feb. 29, 1924

2 Sheets-Sheet 1



Fig. 1.



Fig. 2.



Fig. 3.



Fig. 4.



Fig. 5.

INVENTOR

William P. Witherow  
By George Stebbins, Secretary  
H. C. O. & Co.

Sept. 21, 1926.

1,600,782

W. P. WITHEROW

DIE ROLL AND DIE ROLLING

Filed Feb. 29, 1924

2 Sheets-Sheet 2



INVENTOR  
Wm P. Witherow  
By my attorney  
Wm. P. Witherow  
B. Dyer, St. Louis, Mo.  
Wm. P. Witherow  
Wm. P. Witherow  
Wm. P. Witherow

Patented Sept. 21, 1926.

1,600,782

## UNITED STATES PATENT OFFICE.

WILLIAM P. WITHEROW, OF PITTSBURGH, PENNSYLVANIA, ASSIGNOR TO WITHEROW STEEL COMPANY, OF NEVILLE ISLAND, PENNSYLVANIA, A CORPORATION OF PENNSYLVANIA.

### DIE ROLL AND DIE ROLLING.

Application filed February 29, 1924. Serial No. 695,964.

This invention relates to die rolls and die rolling, and particularly to the formation of matrix portions in die rolls in a way which more closely achieves desired dimensions in the various portions of the product.

I have found that the elongation produced by any particular section of a pair of die rolls, while it varies generally with the percentage of reduction from the leader, will also vary in accordance with the dimensions of a preceding section, particularly if there is a considerable difference in area between such sections.

I believe this to be due to a heretofore uncompensated action of the die rolls on the leader from which the die rolled articles are produced. While ordinarily the ratio of length of a leader to the length of a finished article varies with the ratio of their cross sectional areas, this apparently does not entirely hold true where sudden changes in section of the finished articles are encountered, as in die rolling. Seemingly the metal "piles up" prior to entering the rolls, so that considering only the portion of the leader immediately adjacent the rolls, the finished article is virtually being produced from a leader of greater cross sectional area than the leader which is furnished to the mill. Such being the case, what happens is that if a roll portion designed to produce a larger cross section is encountered, the result will be as though for a very short period the article were being produced from a leader of larger dimensions and such portion would, therefore, be longer than would be expected by the ordinary calculation of lengths by percentage reduction. This is shown very clearly in actual practice, and I have found that when die rolls are designed to compensate for this action, die rolled articles may be produced within exceedingly close dimensions.

The above theory is borne out by the rolling of various articles and I have found that it is even possible to produce a section having portions of a larger cross sectional area than that of the leader supplied to the mill, a section having an excess of as high as 8 to 10 per cent having been produced in regular operation. However, I do not limit myself to this theory.

As above stated, I have found that when

a section of a certain size is followed by a section of larger size it is necessary, if accurate results are to be produced, to shorten the matrix portion which is to produce this larger section. Otherwise, the roll portion will be longer than the calculated size. When conditions are reversed, the action of the preceding section on the succeeding section is also reversed. That is to say, if after rolling a large section we come to a smaller section, the calculated length of the roll matrix portion for such smaller section should be somewhat increased.

In the accompanying drawings which illustrate more or less diagrammatically a few of the applications of my invention—

Figure 1 is a view of a portion of a series of die rolled axle blanks as they come from the mill and while still hot;

Figure 2 is a corresponding view of a trimmed axle blank when cold;

Figure 3 is a developed view of a die roll for producing the strip of Figure 1;

Figure 4 is a section to enlarged scale of a leader from which the strip of Figure 1 is rolled;

Figure 5 is a section to the same scale on line V—V of Figure 1;

Figure 6 is a side elevation of a series of die rolled horseshoe blanks;

Figure 7 is a diagrammatic view showing the roll matrices from which the blank of Figure 6 is produced these, however, being shown as in a straight instead of in a circular manner as in the roll itself;

Figure 8 is a side elevation of a die rolled axle blank; and

Figure 9 is a view similar to Figure 7 and showing in diagrammatic form one of a pair of identical rolls for producing the axle blank shown in Figure 8.

In laying out a pair of rolls for producing the axle blank shown in Figure 2, the length of the article at the rolling temperature is first calculated. A leader of suitable size is then selected and the various portions of the roll matrices are then calculated in view of the reduction for any particular section from such leader. In this particular case the article to be produced is antero-posteriorly symmetrical, and if the matrix portions were calculated solely by taking into account the percentage of reduction from the original

area of the leader, the roll layout would also be symmetrical. As above set forth, however, such a roll will not produce a symmetrical axle blank but instead will produce a blank with one end portion widely varying in dimensions from the other. Figure 1 shows the axle blank with its flash as delivered from the mill, the arrow indicating the direction of rolling. This blank is symmetrical and differs in dimension from the trimmed blank of Figure 2 only by a factor due to temperature difference. If either of these figures, however, is compared with Figure 3 by taking off dimensions with a pair of dividers and making comparison with the dimensions of corresponding matrix portions in the roll layout of Figure 3, it will be found that a number of apparent discrepancies occur. The roll layout of Figure 3 will be found asymmetrical, particularly in the end portions, this variation being due in each case to compensation having been made for the dimensions of a preceding section. For example, in the finished product the distance marked A is 1.7188 inches and the corresponding distance on the hot blank will be such dimension multiplied by a temperature factor. Also, this dimension will be found the same on either end of the blank. However, the roll matrix portion A' in the leading portion of the roll is 1.6744 inches long, while the corresponding portion A'' on the following portion of the roll is only 1.5843 inches long.

These differences in dimensions are due to the difference in cross sectional area of the preceding sections. A section on the chain line  $s-s$  in Figure 1 is only 1.33 square inches in area on the finished product, while a section on the line  $s^1-s^1$  is 2.95 square inches in area. This difference is reflected in the elongation of the article immediately succeeding such section and the dimensions A' and A'' are accordingly varied to compensate for such difference.

Figure 4 shows a cross section of the leader from which the die rolled strip of Figure 1 is produced, and the actual area of such leader is 3.22 square inches. Figure 5 shows the cross section of the largest portion of the axle blank as produced and its area as rolled is 3.48 square inches. It will be seen that this represents an excess over the area of the leader of approximately 8 per cent and bears out my belief that the metal piles up just before it enters the rolls when a small section is being rolled and is squeezed in on an abrupt change from a large section to a smaller one.

To state the matter in another way, the entering speed of the leader is generally near the peripheral speed of the rolls and the delivery speed is considerably in excess, depending upon the amount of reduction. The

difference in entering and delivery speed is termed the forward slippage and would be expected to vary exactly as the difference in area between the leader and the finished section. However, when a change in section of the article is encountered the forward slippage does not exactly correspond to this difference in area as indicated by the difference in the lengths of the portions A' and A''.

Referring to Figures 6 and 7, the dimensions B in the rolled article are each 3.875 inches while the corresponding matrix dimensions B' and B'' are 3.952 and 3.702 respectively. In both of the above described examples it will be seen that symmetrical articles are produced by providing non-symmetrical rolls, or that spaced apart equal portions are rolled by providing unequal roll matrices corresponding to such portions.

Figures 8 and 9 show an axle blank and a straight line diagram of the roll used in its production. In Figure 8 there are indicated two dimensions C and D of substantially the same cross section but preceded by portions of considerably different cross sectional area. For example, the area of the section immediately preceding the portion C is 1.418 square inches, while the maximum section is just ahead of the portion D and is 3.976 square inches. The corresponding dimensions C' and D' vary from the dimensions C and D in different amounts and this is due to the difference in area of the preceding section. In this particular case the ratio of C to C' differs from the ratio of D to D' by a little over 8 per cent, this compensation in the multiplying factor being largely influenced by the difference in area of the preceding sections.

My invention makes it possible to more accurately calculate die rolls since it takes into account an important item in design which has heretofore been neglected with a corresponding expense in the production of accurate and entirely satisfactory die rolls. A large amount of the variation of roll matrix portions from calculated dimensions which have heretofore been made in a more or less haphazard fashion according to the experience of the roll designer is reduced to a definite rule of action, which may even be resolved into a mathematical compensation after the results of a number of similar rolls have been checked and properly applied.

A complete understanding of my invention makes it possible to better select the size of the leader to be employed. As pointed out herein, it is entirely feasible to die roll an article having a maximum section which is larger than the leader from which it is produced. This is of great advantage, since the amount of reduction to be effected is considerably reduced and a

material reduction in the operation and upkeep of the mill may be effected, not only by reducing the strain on the working parts and in the power required, but also by reducing the amount of flash which is produced in such operation.

It will be understood that the dimensions given in the various examples are not fixed and unvarying but are likely to vary in accordance with a large number of other factors, as will be readily appreciated by those skilled in the art. However, they are illustrative of the principles involved and clearly show the importance of making allowance for the dimensions of a preceding section.

While I have illustrated the invention as applied to a few articles commonly produced by die rolling, it will be understood that its application is far beyond these forms and may be applied to other die rolled articles within the scope of the following claims.

I claim:

1. In the method of making die rolls, the steps consisting in varying the dimensions of a roll matrix portion from the theoretical dimensions of such portion as calculated by reduction from the leader, such variations being made to compensate for the change in extrusion effect due to the difference in cross section or shape between a portion preceding the portion in question during the rolling operation, and the portion in question.

2. In the method of making die rolls, the steps consisting in varying the dimensions of a roll matrix portion to compensate for the change in extrusion effect due to the difference in cross section or shape between a portion preceding the portion in question during the rolling operation, and the portion in question.

3. In the method of making die rolls, the steps consisting in compensating for forward slippage in a roll matrix portion by varying the dimensions of a roll matrix portion from the theoretical dimension of such portion as calculated by reduction from the leader to compensate for the change in extrusion effect due to the difference in cross section or shape between a portion preceding the portion in question during the rolling operation and the portion in question.

4. In the method of making die rolls, the steps consisting in varying the ratio of length of a portion to be rolled to the length of the matrix portion for rolling the same from the theoretical ratio calculated in accordance with the percentage of reduction from the leader, such variation being made to compensate for the change in extrusion effect due to the difference in cross section or shape between a portion preceding the portion in question during the rolling operation and the portion in question.

5. In the method of making die rolls for rolling antero-posteriorly symmetrical articles of varying cross section, the steps consisting in forming pairs of corresponding matrix portions in the roll to produce the symmetrical articles and varying the dimensions of a pair of such matrix portions one from the other to compensate for the change in extrusion effect due to the difference in cross section or shape between portions preceding the portions in question during the rolling operation.

6. In the method of making die rolls for the production of articles having a pair of equal portions connected by an intermediate portion of different dimensions, the steps consisting in forming matrix portions of unequal dimensions for the production of such equal portions, the unequal dimensions being made to compensate for the change in extrusion effect due to the difference in cross section or shape between the second of such equal portions produced by the die rolls and the intermediate portion.

7. In the method of making die rolls for rolling articles of varying cross section and having a plurality of spaced apart equal portions, separated by an intermediate portion of different cross section, the steps consisting in providing unequal roll matrices corresponding to such spaced apart portions, the difference in dimensions in such roll matrices being made to compensate for the change in extrusion effect due to the difference in cross section or shape between the portions preceding such equal portions during the rolling operation.

8. As a new article of manufacture, a die roll having a matrix portion whose dimensions vary from the theoretical dimensions to compensate for the change in extrusion effect due to the difference in cross section or shape between a portion preceding the portion in question during the rolling operation and the portion in question.

9. As an article of manufacture, a die roll having a matrix portion whose length varies from the length calculated in accordance with reduction from the leader, such variation being made to compensate for the change in extrusion effect due to the difference in cross section or shape between a portion preceding the portion in question during the rolling operation and the portion in question.

10. As an article of manufacture, a die roll for the production of antero-posteriorly unsymmetrical articles, said roll having unsymmetrical matrix portions, said matrix portions varying from one another to compensate for the change in extrusion effect due to the difference in cross section or shape between portions preceding the portions in question during the rolling operation.

11. As an article of manufacture, a die for the change in extrusion effect due to the difference in cross section or shape between portions preceding the said spaced 10 apart portions during the rolling operation. In testimony whereof I have hereunto set my hand.

WILLIAM P. WITHEROW.